

H. E. TIFFANY.

PROCESS OF ELIMINATING AND RECOVERING ACIDS OR METALLIC SALTS.

APPLICATION FILED JAN. 5, 1916.

1,226,279.

Patented May 15, 1917.



Harold E. Tiffany Inventor

By E. C. Brandenburg  
His Attorney

# UNITED STATES PATENT OFFICE.

HAROLD E. TIFFANY, OF NEWARK, DELAWARE, ASSIGNOR TO THE CONTINENTAL FIBRE COMPANY, OF NEWARK, DELAWARE, A CORPORATION OF DELAWARE.

## PROCESS OF ELIMINATING AND RECOVERING ACIDS OR METALLIC SALTS.

1,226,279.

Specification of Letters Patent.

Patented May 15, 1917.

Application filed January 5, 1916. Serial No. 70,477.

To all whom it may concern:

Be it known that I, HAROLD E. TIFFANY, a citizen of the United States, residing at Newark, in the county of Newcastle and 5 State of Delaware, have invented certain new and useful Improvements in Processes of Eliminating and Recovering Acids or Metallic Salts, of which the following is a specification.

10 My invention relates to an improved process of eliminating acids or metallic salts, such as chlorid of zinc, used in the manufacture of certain fibrous materials, and in recovering same.

15 Among other things, it consists in the application of electrolysis or an electrolytic method to the washing or puring out of fiber or similar material in sheet, tube, or other form for the elimination of any metallic salt, such as, for instance, zinc chlorid commonly used in the manufacture of fiber, or an acid that will gelatinize and harden cellulose in a way similar to zinc chlorid. 20 Fiber or similar material washed or pured out by my improved electrolytic method is more thoroughly cleansed than has hitherto been possible, and in less time, and therefore more economically, and, as practically all the solution is recovered, no extra cost 25 is incurred in consequence.

In the accompanying drawings:—

Figures 1, 2 and 3 are views showing a few of many forms of tanks containing an electrolyte with positive and negative electrodes, and showing the sheets of fiber arranged therein.

30 The most approved method now in use of making vulcanized fiber is to wind up layers of paper, each layer being saturated with zinc chlorid. My method is not limited to the use of zinc chlorid, but contemplates the use of any metallic salt, or in fact any acid that might be used for gelatinizing cellulose. The action of metallic salt or acid 35 used does not harden the cellulose at once, because it is the cellulose in the paper that the acid affects, the theory being that paper must be used containing as much cellulose as possible, as for instance cotton paper, 40 which is then passed through the bath of acid or metallic salt that gelatinizes or softens the cellulose. Continually winding one sheet upon another in this condition sticks the material together, but the cellulose is not

hardened, and the material itself does not 55 become hard until all the acid or metallic salt or zinc chlorid used is washed out and the material is dried.

The present method of washing has been to first place the sheets of fiber in a tank 60 containing either clear water, or preferably a weaker solution of zinc chlorid, usually about 25° B. and then transfer it from tank to tank through a zinc chlorid solution of diminishing strength, until at last it reaches 65 pure water, and stays there until all possible traces of the zinc chlorid solution originally used are washed or soaked out, and the product is commercially pure and ready 70 to dry and be finished in the usual manner. 70

While it would be perfectly possible to place the sheets in pure water at the start, yet it is economical to use the zinc chlorid solution over and over again, and consequently it is customary to provide a long 75 series of tanks, pure water being supplied at one end of the series and pumped forward from tank to tank, while the fiber is started at the other end of the series and moved from tank to tank toward the pure 80 water. In other words, the fiber is moved all the time toward fresh water, and the fresher water is pumped from tank to tank as it becomes stronger and stronger with the chlorid of zinc solution, until finally 85 when the solution at the farthest end reaches a strength of about 25° to 30° B. it is pumped into other tanks, where by boiling, the excess water is evaporated and the strength of the zinc chlorid raised to a point 90 where it can be used for the first solution into which the fiber is placed for its original saturation with the zinc chlorid.

The trouble with this process of washing is that it involves a large amount of labor 95 in moving the fiber from tank to tank, and above all it is a long, slow process, requiring from three to five weeks to wash or pure out sheets of fiber only one-eighth of an inch in thickness, and correspondingly 100 longer where the sheets are of greater thickness.

In my present process, I utilize the well-known method of electrolysis or electrolytic action, which, briefly described, comprises 105 the action of a direct current of electricity upon an electrolyte made of any solution containing an acid and a metal, or a purely

acid solution, or in fact any solution that will carry an electric current. It is well known that the application of a direct electric current to any of these solutions results in its being separated into its component parts. As for instance, in a tank of water that is pure, or nearly so, the fiber is placed on being taken from the making machine, in which condition it is saturated with the zinc chlorid solution, this zinc chlorid solution becoming readily absorbed into the water and resulting quickly in changing the water from ordinary pure water to a weak solution of zinc chlorid, thereby making it conductive to direct current.

It is perfectly obvious that various elements might be used in the way of electrodes. As shown in the drawings, on one side of the tank 1, into which these sheets 20 of fiber are placed, zinc or other suitable metal which is the negative electrode is placed, and on the other side a sheet or bolt of lead 3 might be employed, as shown in Fig. 1; or, of course, carbon or any other 25 material could be used to form the positive electrode. To each electrode is attached a wire 4 and 5 respectively, connected to the source of direct current, and the current is then turned on, and at once electrolysis or 30 electrolytic action takes place. This causes the zinc chlorid to separate from the fiber and into its component parts, the zinc depositing itself upon the negative electrode 2 as metallic zinc and the muriatic acid collecting around the positive electrode and in 35 solution with the water.

By this method of washing or puring out, I have found by actual test that a sheet of fiber one-eighth of an inch in thickness may 40 be entirely cleansed in about twelve hours, so that the fiber thus treated will become a perfect insulator instead of a conductor of electricity, which it would be if any considerable vestige of the zinc or metallic salts 45 remained in its composition.

As an alternative, if desired, each sheet of fiber may be connected to the positive and negative electrode by making the bottom of the tank one electrode, as shown in Fig. 3, 50 and connecting the sheets together mechanically in some way as illustrated. In fact, any arrangement of electrodes and connection thereto may be used that is found most convenient to the particular situation of the tank, or the size and shape of the sheet of fiber to be pured out. The same thing applies to tubular or other shapes that are made of fiber. In fact, the fiber sheets when 55 saturated with the zinc chlorid or other metallic salts may form the positive electrodes themselves, and remain so until the last vestige of zinc chlorid is decomposed and eliminated therefrom.

After I pure out a tank of fiber by my 60 improved process, and the fiber is removed,

there is left in the tank an acid solution, the metallic zinc being separated and deposited in the bottom. I therefore pump the acid solution off, and concentrate it by evaporation in the presence of the metallic zinc, the two again go into solution, and form zinc-chlorid, which is available for use again in the preliminary stages of manufacture. The zinc chlorid is thus reclaimed as in the old method.

As shown in Fig. 3, the negative electrode might be in the bottom in the form of a slotted or perforated or grated plate, or an ordinary zinc plate might be placed on the bottom.

Any acid remaining on the surface of the fiber at the conclusion of the process may be readily rinsed off.

It may not be necessary to connect each fiber sheet mechanically.

The voltage and amperage may be varied to suit conditions, and also the thickness and number of sheets in the tank, as previously suggested, and the temperature of the solution; but the higher the voltage, the quicker 90 the action, although if too high, overheating may result in damage to the fiber. My preference is a low voltage to prevent overheating, but a relatively high voltage may be used if the solution is cooled either by 95 circulating coils or by changing the water from time to time.

This process may be applied to thinner fiber that is made continuously in rolls, substantially as described, that is by the use 100 of direct current to the puring tank, thus making fewer tanks necessary.

It may also be applied to any process of manufacture involving the use of conductive solution, and the necessity of removing it 105 from the finished product.

I claim:

1. The improved method of washing and puring out fiber or similar substance containing metallic salts or acid, which consists in subjecting the material to electrolytic action.

2. The herein-described method or process of eliminating the metallic salts or acids used in the hardening of fiber, which consists in subjecting the material to electrolysis.

3. The herein-described method or process of eliminating the metallic salts or acids used in the hardening of fiber, which consists in subjecting the material to electrolytic action by placing the fiber saturated with the hardening material in an electrolyte and passing a current through it.

4. The herein-described method or process 125 of eliminating the metallic salts or acids used in the hardening of fiber, which consists in subjecting the material to electrolytic action by placing the fiber saturated with the hardening material in an electro-

75

80

85

90

95

100

105

110

115

120

125

130

lyte, passing a current through it, and employing the fiber thus saturated as one of the electrodes.

5. The herein-described method or process of eliminating metallic salts or acids used in the treatment of certain fibrous materials and in recovering same, which consists in submerging the fibrous materials in a bath of acid or metallic salts, which gelatinizes

or softens the cellulose therein, then subjecting the material under treatment to electrolytic action, whereby to remove and recover the acid or metallic salts, and finally drying the fibrous material treated, which then results in the hardening of the latter. 10 15

In testimony whereof I affix my signature.

HAROLD E. TIFFANY.